

3,401,054  
FORMATION OF COATINGS ON  
GERMANIUM BODIES

John George Wilkes, Hatch End, Middlesex, England, assignor to The General Electric Company Limited, London, England  
No Drawing. Filed Sept. 3, 1965, Ser. No. 485,078  
5 Claims. (Cl. 117—201)

In British patent specification No. 976,559 we have 10 disclosed that it is possible to form on a germanium body a coating of germanium dioxide having a tetragonal crystal structure, such a coating being usable for certain purposes connected with the technology of semiconductor devices.

It is an object of the present invention to provide a method of forming such a coating, alternative to the methods described in the aforesaid application.

According to the invention, in a method of forming on a germanium body a coating of germanium dioxide having a tetragonal crystal structure, the body is heated above 400° C. while exposed to an oxidising atmosphere containing water vapour, the total pressure of said atmosphere being at least 30 kgs./cm.<sup>2</sup>.

The results obtained, in respect of the thickness and quality of the resultant coating, when using such a method depend on a number of factors. Firstly, it may be observed that the best results in respect of coherence of the coating are obtained when using relatively high temperatures (say above 600° C.); with such temperatures, the results are not very dependent on the total pressure of the oxidising atmosphere provided this exceeds the minimum indicated above. The results are, however, very dependent on the amount of water vapour present in the atmosphere; other things being equal, an increase in the amount of water vapour results in an increase in the thickness of the coating and also causes the coating to have a more granular nature. The thickness of the coating is also dependent on the time and temperature of the heating, increasing with an increase of either of these factors, while an increase in the time of heating also results in an improvement in the coherence of the coating.

It will be appreciated that when using a method according to the invention in the manufacture of semiconductor devices, it will normally be required to provide a good coherent coating of well controlled thickness. To this end, it will normally be desirable to carry out the method at a temperature above 600° C., and to choose the water vapour content of the oxidising atmosphere so as to obtain a coating of the desired thickness in a time which is sufficiently short to be convenient from the point of view of a manufacturing process but at the same time sufficiently long to ensure that the coating has the required degree of coherence; it may be noted that a time of about 20 hours will normally be suitable having regard to these considerations.

It will normally be convenient to use an atmosphere consisting essentially of oxygen and water vapour only, although in some cases these active constituents of the atmosphere may be diluted with an inert gas such as nitrogen.

One method of performing the invention will now be described by way of example.

In this method a germanium body, which has been chemically cleaned in conventional manner, is placed in a steel high pressure vessel which has an internal volume of about 100 cc. and which is lined with platinum to prevent contamination of the contents. A controlled amount of water, having a volume in the range 0.1–0.5 cc., is introduced into the vessel, and the vessel is then filled 70 with oxygen at a pressure in the range 100–150 kgs./cm.<sup>2</sup>

and sealed. The sealed vessel is heated in a suitable furnace to a temperature of about 700° C., being maintained at this temperature for about 20 hours and then allowed to cool to room temperature. During the heating the oxygen pressure within the vessel increases to about three times its initial value; the amount of water introduced into the vessel is such that the partial pressure of water vapour within the vessel is small compared with that of the oxygen.

As a result, the germanium body has formed on it a coherent adherent coating of germanium dioxide having a tetragonal crystal structure; the thickness of the oxide coating may be varied over a range of approximately one to twenty microns by choice of the precise value, within the range indicated above, of the volume of water introduced into the vessel. The oxide has crystal lattice unit cell dimensions, determined by X-ray analysis, as follows:

| A.   |       |
|------|-------|
| 20 a | 4.396 |
| c    | 2.862 |
| c/a  | 0.651 |

that is it is of the form denoted T(I) in British patent specification No. 976,559.

I claim:

1. A method of manufacturing a germanium body having formed on its surface a coherent adherent coating of germanium dioxide having a tetragonal crystal structure, which includes the steps of exposing a germanium body, initially free from any surface coating, to an oxidizing atmosphere containing water vapor, the total pressure of said atmosphere being at least 30 kilograms per square centimeter, and heating the said body at a temperature above 400° C., while the body is exposed to said atmosphere.

2. A method according to claim 1 wherein the said atmosphere consists essentially of oxygen and water vapor, the partial pressure of the water vapor being small compared with that of the oxygen.

3. A method according to claim 1 wherein the germanium body is heated, while exposed to the said atmosphere, at a temperature above 600° C.

4. A method according to claim 3 wherein the said heating of the germanium body is continued for about 20 hours.

5. A method of manufacturing a germanium body having formed on its surface a coherent adherent coating of germanium dioxide having a tetragonal crystal structure, which includes the steps of placing a germanium body in a steel pressure vessel lined with platinum, then introducing into the said vessel a volume of water in the range of 0.1% to 0.5% of the internal volume of the vessel, then filling the vessel with oxygen at a pressure in the range of 100 to 150 kilograms per square centimeter and sealing the vessel, then heating the sealed vessel to a temperature of 700° C. and maintaining it at this temperature for about 20 hours, and then allowing the vessel to cool to room temperature before withdrawing the coated germanium body therefrom.

## References Cited

### UNITED STATES PATENTS

|           |        |                 |           |
|-----------|--------|-----------------|-----------|
| 3,298,875 | 1/1967 | Schink          | 117—201 X |
| 3,340,163 | 9/1967 | Bradshaw et al. | 117—201 X |
| 3,342,619 | 9/1967 | Chu             | 117—201   |

### FOREIGN PATENTS

|         |         |            |
|---------|---------|------------|
| 219,126 | 12/1958 | Australia. |
|---------|---------|------------|